

## UNITED STATES PATENT OFFICE

GREGORY J. COMSTOCK, OF PITTSBURGH, PENNSYLVANIA, ASSIGNOR TO FIRTH-STERLING STEEL COMPANY, OF MCKEESPORT, PENNSYLVANIA, A CORPORATION OF PENNSYLVANIA

## COMPOSITION OF MATTER

No Drawing.

Application filed April 9, 1928. Serial No. 268,390.

The present invention relates broadly to an improved composition of matter and more particularly to a composition comprising the combination of a cutting agent or cutting agents of abrasive characteristics with a binding agent.

I have found that certain materials, which are hereinafter referred to as cutting agents, when held together by indefinite percentages of a suitable binder, provide a composition of matter having such characteristics as to render them suitable for a wide variety of purposes. Within the class of cutting agents are included such materials as silicon carbide, tungsten carbide, and vitrified zirconium oxide, these materials being considered as cutting or abrasive agents due to their extreme hardness. The utility of the invention, however, is not limited necessarily with respect to the particular cutting agent employed, although those referred to give desirable results in accordance with the methods hereinafter described.

While the present invention adapts itself to the use of a wide variety of binders, I prefer to utilize a metallic binder comprising an alloy steel. By "alloy steel" I mean an iron-carbon alloy containing minor amounts of elements such as silicon, sulphur, phosphorus, and manganese, together with an alloying element. Within the classification designated by this title, I include preferably manganese steels, high carbon-high chrome steels, oil-hardening steels, so-called stainless steels and irons, chrome vanadium steels, and high carbon chrome nickel steels. Each one of these alloys possesses characteristics when utilized in accordance with the present invention which impart desirable properties to the resulting product. The particular selection of the alloy steel is dependent upon the special use to which the product is to be applied.

I have found that manganese steels as a binding agent are particularly desirable by reason of their tough nature and ability to tenaciously adhere to the particles of the cutting agent or agents. Such steels have also an extremely high resistance to abrasion.

In addition to the above, manganese steels possess the faculty of acquiring hardness upon slow cooling. This is directly the opposite, for example, of high speed steels, which must be rapidly cooled, as by quenching, in order to impart the desired hardness thereto.

A typical example of manganese steel which may be utilized in accordance with this invention is the following:

## Typical example

| Carbon             | Silicon       | Manganese       | Sulphur | Phosphorus | Iron    |
|--------------------|---------------|-----------------|---------|------------|---------|
| 1.00%<br>.85-1.25% | .25%<br>1.25% | 15.00%<br>3-20% | .030%   | .040%      | Balance |

The high carbon-high chrome steels likewise have certain characteristics which peculiarly adapt them to use with cutting agents of the character herein contemplated. Like the manganese steels, they have a high resistance to abrasion. In addition to this, they, and the product resulting from their use, may be hardened in air, oil or water, thereby giving to such a steel a broad adaptability.

The following tables give both typical analyses and the usual variations of high carbon-high chrome steels as herein contemplated:

|              | Typical analysis |                       | Usual variations |
|--------------|------------------|-----------------------|------------------|
|              | Type A           | Type B                |                  |
| Carbon       | Per cent<br>1.50 | Per cent<br>1.20-1.80 |                  |
| Silicon      | .25              |                       |                  |
| Manganese    | .35              |                       |                  |
| Sulphur      | .030             |                       |                  |
| Phosphorus   | .030             |                       |                  |
| Chromium     | 11.50            | 10.00-14.00           |                  |
| Vanadium     | 1.00             | .75-1.25              |                  |
| Molybdenum   | 1.00             | .75-1.25              |                  |
| Balance—iron |                  |                       |                  |

## Type B

|              | Per cent | Per cent |
|--------------|----------|----------|
| Carbon       | 2.25     | 2-2.50   |
| Silicon      | .30      |          |
| Manganese    | .30      |          |
| Sulphur      | .030     |          |
| Phosphorus   | .030     |          |
| Chromium     | 12.50    | 10-14.00 |
| Balance—iron |          |          |

## Type B

Oil-hardening steels possess the property of displaying a minimum dimensional change as a result of heat treatment. This renders them particularly applicable as a binder of the abrasive particles, in that the minimizing of the disposition to contract or expand greatly reduces the tendency to weaken the product by loosening the hold of the binding material upon the abrasive grains, through movement or permanent distortion. There are two general types of oil-hardening steels

which may be used in this way, examples of which are shown in the following tables:

|    | Typical analysis                                                                                                                                                                                                                                                                                                                                                                        | Usual variations                                               | Type D                                                                |          | 70 |
|----|-----------------------------------------------------------------------------------------------------------------------------------------------------------------------------------------------------------------------------------------------------------------------------------------------------------------------------------------------------------------------------------------|----------------------------------------------------------------|-----------------------------------------------------------------------|----------|----|
|    |                                                                                                                                                                                                                                                                                                                                                                                         |                                                                | Per cent                                                              | Per cent |    |
| 5  |                                                                                                                                                                                                                                                                                                                                                                                         |                                                                |                                                                       |          |    |
| 10 | Carbon.....<br>Silicon.....<br>Manganese.....<br>Sulphur.....<br>Phosphorus.....<br>Balance—iron.                                                                                                                                                                                                                                                                                       | Per cent<br>.80<br>.25<br>1.60<br>.030<br>.030                 | Per cent<br>.70 to 1.00<br>1.40 to 1.80                               |          |    |
| 15 |                                                                                                                                                                                                                                                                                                                                                                                         |                                                                |                                                                       |          |    |
| 20 | Carbon.....<br>Silicon.....<br>Manganese.....<br>Sulphur.....<br>Phosphorus.....<br>Chromium.....<br>Tungsten.....                                                                                                                                                                                                                                                                      | Per cent<br>.80<br>.25<br>1.50<br>.030<br>.030<br>.50<br>.50   | Per cent<br>.70 to 1.00<br>1.40 to 1.80<br>.25 to 1.00<br>.25 to 1.00 |          |    |
| 25 | The so-called stainless steels and irons possess the well recognized property of resistance to corrosion as well as a tendency to retain their physical strength at fairly high temperatures. Their high chromium content also renders them resistant to abrasive action and the combination of these properties makes them a desirable metal binding agent for use in this connection. |                                                                |                                                                       |          |    |
| 30 | Tungsten carbide is not susceptible to corrosion, and therefore, when suitably united with a non-corrosive binding material, the resulting product is also resistant to corrosion. The use of stainless steels and alloys is therefore extremely desirable. Examples of the types which may be used in this connection are listed in the following tables:                              |                                                                |                                                                       |          |    |
| 40 |                                                                                                                                                                                                                                                                                                                                                                                         |                                                                |                                                                       |          |    |
| 45 | Carbon.....<br>Silicon.....<br>Manganese.....<br>Chromium.....<br>Sulphur.....<br>Phosphorus.....<br>Balance—iron.                                                                                                                                                                                                                                                                      | Per cent<br>.35<br>.20<br>.30<br>13.50<br>.030<br>.030         | Per cent<br>.25 to .45<br>11.00 to 14.00                              |          |    |
| 50 |                                                                                                                                                                                                                                                                                                                                                                                         |                                                                |                                                                       |          |    |
| 55 | Carbon.....<br>Silicon.....<br>Manganese.....<br>Chromium.....<br>Sulphur.....<br>Phosphorus.....<br>Balance—iron.                                                                                                                                                                                                                                                                      | Per cent<br>.65<br>.25<br>.35<br>16.50<br>.030<br>.030         | Per cent<br>.60 to .85<br>16.00 to 18.00                              |          |    |
| 60 |                                                                                                                                                                                                                                                                                                                                                                                         |                                                                |                                                                       |          |    |
| 65 | Carbon.....<br>Silicon.....<br>Manganese.....<br>Chromium.....<br>Sulphur.....<br>Phosphorus.....<br>Nickel.....<br>Balance—iron.                                                                                                                                                                                                                                                       | Per cent<br>.18<br>.30<br>.40<br>18.00<br>.030<br>.030<br>8.00 | Per cent<br>.14 to .25<br>16.00 to 20.00<br>6.00 to 10.00             |          |    |

| Type D          |          | 70             |
|-----------------|----------|----------------|
| Per cent        | Per cent |                |
| Carbon.....     | .10      |                |
| Silicon.....    | .30      |                |
| Manganese.....  | .40      |                |
| Chromium.....   | 12.00    | 11.50 to 13.50 |
| Sulphur.....    | .030     |                |
| Phosphorus..... | .030     |                |
| Nickel.....     | .40      | .00 to 1.00    |

Chrome vanadium steels are characteristically hard and tough and possess a remarkable high wear-resisting quality, and are strongly coherent, making them particularly applicable as a metal binding agent for the abrasive of this product. When properly heat treated, they display a high tensile strength coupled with good elastic properties. A steel of the type which I use in this product is exemplified in the following table:

|                | Typical analysis | Usual variations | 90 |
|----------------|------------------|------------------|----|
|                | Per cent         | Per cent         |    |
| Carbon.....    | .30              | .30 to .45       |    |
| Silicon.....   | .25              |                  |    |
| Manganese..... | .25              |                  |    |
| Chromium.....  | 3.25             | 3.00 to 4.00     |    |
| Vanadium.....  | .60              | .30 to 1.25      | 95 |

I have also found that a material, the character of which is in the zone between that of cast iron and a true steel possesses desirable attributes when used as a binding agent. 100 When united with the abrasive according to this invention, this material is exceptionally hard and resistant to the action of abrasion under heat and is at the same time susceptible to considerable deformation in the hot condition. Thus it combines several desirable properties which make it specially suitable for use as a binding agent.

A typical example of such a binding agent is shown in the following table:

|                 | Typical analysis | Usual variations |     |
|-----------------|------------------|------------------|-----|
|                 | Per cent         | Per cent         |     |
| Carbon.....     | 1.90             | 1.70 to 2.20     | 115 |
| Silicon.....    | .60              | .40 to .80       |     |
| Manganese.....  | .35              | .20 to .40       |     |
| Phosphorus..... | .06              |                  |     |
| Sulphur.....    | .80              |                  |     |
| Nickel.....     | .90              | .5 to 1.00       |     |
| Chromium.....   | 1.18             | .75 to 1.60      |     |

In carrying out the present invention, I preferably take the desired cutting agent or mixture of cutting agents and pulverize the same to very finely divided condition, preferably to a fineness which will pass through a two hundred mesh screen. The same procedure is followed with the binding agent.

The cutting agent or agents and the binding agent having been reduced to the desired fineness, they are mixed together in 130

varying proportions, depending upon the characteristics which are desired in the final composition. Where brittleness of the product is no limiting factor, small percentages of binder may be used, but where strength and resistance to shock are required, larger percentages of binder must be present. It is notable that where the binder is increased, the cutting or abrading value of the abrasive and likewise the cutting or abrading value of the product is necessarily decreased, due to the relatively greater dispersion of the cutting particles. For example, in cases of the character first referred to, I may utilize as high as ninety-five percent of the cutting agent or cutting agents with desirable results, while in the latter case, the binding agent may be decreased up to ninety-five percent or even higher.

20 In some cases, I have found that beneficial results are obtained by the mere addition of a trace of the cutting agent to a standard alloy steel of the character herein recited, and especially manganese alloys.

25 In some cases, it is desired to provide a composition of matter of such nature that it lends itself to shaping and deforming by hot working. In such cases, I utilize not less than thirty, and preferably not less than fifty,

30 30 percent of the binding agent, although variations in this amount may be made one way or the other, while retaining some degree of workability.

#### Example I

35 A specific example of a composition suitable for use in the production of tools, such as drawing dies, extrusion dies, high speed cutting tools, such as bits, shapers, drills, cutters, saws, and the like, is as follows:

40 Tungsten carbide, 87.00%; 13.00% of a manganese steel as herein referred to.

#### Example II

45 As a specific example of a composition of brittle character useful for the production of dressing tools, metal grinding stones, knife sharpeners, and the like, I refer to the following:

50 Tungsten carbide, 95.00%, 5% of a manganese steel as herein referred to.

#### Example III

55 Where it is important that the resulting product have workable characteristics, I have found that a composition in accordance with the following gives desirable results:

Tungsten carbide, 30.00%; Manganese steel, as herein referred to, 70.00%.

Having determined upon the proper composition depending upon the character which the resulting product is to have for its specific application, I may proceed in accordance 65 with any of four different methods. The

first of these involves the pressing to shape followed by fusing without any subsequent pressure; the second involves the pressing to shape followed either in sequence or simultaneously by heat and pressure; the third involves the application of heat and pressure simultaneously without any preliminary pressing; while the fourth involves the application of heat followed by the application of pressure, without any preliminary pressing.

70 In accordance with the first method, which will hereinafter be referred to as the cold compacting method, I preferably form a paste by using gum tragacanth in the amount of one ounce of the gum tragacanth to a pint of water and add this paste to the mixture of cutting agent or cutting agents and binding agent, in the ratio of about one-half of one percent by weight. This mixture is then subjected to pressure while cold, the pressure preferably being of the order of one hundred fifty tons to the square inch. This produces a closely compacted mixture which is then subjected to a temperature sufficiently high 75 to melt the binding agent and cause it to actually flow around the cutting agent or cutting agents, so that upon cooling, such agent or agents will be substantially uniformly dispersed or distributed throughout the product with each particle firmly bonded in the binding material, which in this case forms a metal matrix.

80 In the second method, the preliminary steps of forming a paste-like mixture and pressing the same are followed. Thereafter this mixture is subjected to heat to fuse the binding agent, and either simultaneously with the application of the heat, or subsequently thereto while the mixture is still 85 hot, is subjected to pressure.

85 In the third method, the preliminary compacting is dispensed with, the mixture being subjected in a suitable mold to heat and pressure simultaneously.

90 In accordance with the fourth method, which also obviates the necessity for any preliminary cold pressing, the mixture is subjected to the desired temperature conditions, and thereafter, while still hot, is subjected to 95 pressure.

95 The second, third, and fourth methods have the advantage of providing pressure at such a time as to tend to close up any pores which may have formed under the heat treatment 100 by reason of the volatilization of any of the ingredients. Also, these three last mentioned processes require a materially lower pressure, pressures as low as from seventy-five to one hundred fifty pounds per square 105 inch producing satisfactory results with some mixtures.

110 In heating, in each of the methods above referred to, I prefer to employ temperatures in the neighborhood of 2800° F., although it

will be obvious that this temperature depends on the particular metallic binder employed and may vary within fairly wide limits. During the heating, suitable precautions

5 must be taken to prevent oxidation of the product. This may be accomplished, for example, by heating in a reducing atmosphere of hydrogen.

10 In all cases where a paste has been formed by the use of gum tragacanth, the application of heat volatilizes the same from the mixture.

15 The hardness of the composition in accordance with my invention is such that once it has been produced, it does not lend itself to grinding or cutting by known methods. It is therefore desirable, in case the proportions are not such as to produce a workable product, i. e., a product lending itself to shaping or deformation when heated to a suitable 20 temperature, to subject the mixture to pressure in a mold of the desired configuration of the finished article. In this manner, a completed article, such as a tool, can be formed directly from the mixture.

25 While I have herein referred to certain specific types of alloy steels for the purpose of giving a clear understanding of my invention, it will be understood that the particular analyses set forth are given by way of illustration only and not by way of limitation.

30 Throughout the foregoing description where I have referred to tungsten carbide, I preferably utilize a carbide having approximately six percent of carbon combined with 35 the tungsten. I have found that the other carbides of tungsten produce compositions of materially different characteristics.

35 While in the specific examples herein given I have referred to the use of tungsten carbide, this being the present preferable cutting agent, either alone or in conjunction with other cutting agents of the character herein referred to, it will be understood that the other cutting agents may be utilized to replace or partly replace the tungsten carbide, 45 the results obtained varying with the characteristics of the particular cutting agent utilized.

40 It will be understood by those skilled in the art that the present invention, according to the best of our present knowledge, results purely in a mechanical mixture or aggregate, the different materials utilized not combining chemically to any material degree, 55 under the temperature and pressure conditions to which they are subjected.

50 It is to be understood that I have described the present preferred embodiment of my invention, but that it is not limited except as 60 required by the appended claims.

I claim:

65 1. A sintered aggregate comprising finely divided particles of tungsten carbide embedded in a matrix of alloy steel, the tungsten carbide constituting the major part of

the aggregate, the alloy steel containing about 15% manganese and about 1% carbon, and having the property of hardening upon slow cooling.

2. A sintered aggregate comprising finely divided particles of tungsten carbide embedded in a matrix of alloy steel, the tungsten carbide constituting the major part of the aggregate, the alloy steel containing about 3-20% manganese and about .65-1.25 carbon.

70 75 In testimony whereof I have hereunto set my hand.

GREGORY J. COMSTOCK.

80

85

90

95

100

105

110

115

120

125

130

**CERTIFICATE OF CORRECTION.**

**Patent No. 1,815,613.**

**Granted July 21, 1931, to**

**GREGORY J. COMSTOCK.**

**It is hereby certified that error appears in the printed specification of the above numbered patent requiring correction as follows: Page 1, line 9, for the word "indefinite" read definite; and that the said Letters Patent should be read with this correction therein that the same may conform to the record of the case in the Patent Office.**

**Signed and sealed this 1st day of September, A. D. 1931.**

**(Seal)**

**M. J. Moore,  
Acting Commissioner of Patents.**